

## UNITED STATES PATENT OFFICE.

FRANKLIN V. CHANEY, OF BOSTON, MASSACHUSETTS, ASSIGNOR TO CHATON FIBRE COMPANY, OF BOSTON, MASSACHUSETTS, A CORPORATION OF MASSACHUSETTS.

## LEATHERBOARD FELT.

No Drawing.

Application filed March 8, 1923. Serial No. 623,749.

*To all whom it may concern:*

Be it known that I, FRANKLIN V. CHANEY, a citizen of the United States, residing at Boston, in the county of Suffolk and State 5 of Massachusetts, have invented certain new and useful Improvements in Leatherboard Felt; and I do hereby declare the following to be a full, clear, and exact description of the invention such as will enable others 10 skilled in the art to which it appertains to make and use the same.

The present invention relates to an improvement in leatherboard felt.

The object of the invention is to produce 15 a compressible, resilient felt adapted for use in the manufacture of dust guards for railway car axle boxes, and for other purposes, at a low cost.

Heretofore dust guards have very generally 20 been made of wood, but such dust guards have been unsatisfactory owing to their frequent breakage and their inefficiency as dust guards. It has been proposed to use hair felt for dust guards, but such a dust 25 guard is expensive and the interstitial spaces being large ordinarily supply an excess of oil to the axle.

The present invention consists of a leatherboard felt preferably made on a paper 30 making machine of the type known as the wet machine, comprising 40% leather fibre, 20% mixed paper fibre or paper pulp, and 30% goat or cow hair or other form of coarse animal or vegetable fibre, and 10% binder. The material is manufactured according to the ordinary paper board process. The coarse fibre is put in the beater after the 35 leather fibre and paper fibre are beaten up to a proper degree of fineness. The binder is added to the contents of the beater, resin size first being beaten in until it is thoroughly 40 mixed throughout the mass, whereupon aluminum sulphate is added to precipitate the resin size in the form of a sodium resinate. The felt is made from the stock thus 45 prepared on the usual paper machine in the usual manner with this exception, that the pressure of the make roll employed is less than that ordinarily employed in making 50 leatherboard, and more than that employed in making the felt described in the Clapp Patent No. 1,427,263, dated August 29, 1922.

The proportions of the ingredients may be varied somewhat. Thus, the leather fibre

may be increased from 40% to 50% when it is desired to produce a felt having smaller interstitial spaces. The paper pulp ingredient may be as low as 15% or as high as 25%. The coarse fibre constituent may be increased when it is desired to increase the interstitial spaces of the felt. The felt that forms the subject of this invention is a compressible, resilient felt board, the voids or interstitial spaces of which are such as to enable it to conduct and lift by capillarity the required amount of oil for dust guard purposes. When the felt is to be used for other purposes, or in cases where a lesser or greater capacity to lift the oil by capillarity is desired, the proportions of the ingredients may be changed as above set forth. The binder stiffens and gives rigidity to the product, which otherwise would be a soft, almost flocculent, lightly adherent mass of small tensile strength and so weak as to be easily broken in handling. The binder contributes to the value of the product for use as a dust guard material by reason of its reduction of the interstitial spaces while at the same time maintaining a vigorous, self-supporting, stiff felt.

A mixture of leather fibre and paper fibre alone produces too firm a product having voids or interstitial spaces too small to fill the requirements of a dust guard, but the present leatherboard felt is desirable because it permits the capillary absorption of the oil for the purpose of lifting the oil from the bottom of the journal box to the journal. Such leatherboard would not be satisfactory material for use in the manufacture of dust guards.

With the present prices of leather fibre and waste paper from \$10. to \$15. per ton, and cow or goat hair from \$80. to \$120. per ton, it is apparent that this product can be made very cheaply, and this is an extremely important feature of the present invention.

Having thus described the invention, what is claimed is:

1. A leatherboard felt comprising 40% leather fibre, 20% mixed paper fibre, 30% coarse animal or vegetable fibre, and 10% binder.

2. A resilient felt suitable for dust guards for railway car axle boxes susceptible of compression in thickness by moderate pressure, comprising leather fibre, paper fibre,

coarse animal or vegetable fibre, in which the animal or vegetable fibre operates to distend the leather and paper fibre and form interstitial oil conducting spaces.

5. 3. A resilient felt suitable for dust guards for railway car axle boxes susceptible of compression in thickness by moderate pres-

sure, comprising from 40% to 50% leather fibre, from 15% to 25% paper fibre, from 30% to 50% coarse animal or vegetable fibre, <sup>10</sup> in which the animal or vegetable fibre operates to distend the leather and paper fibre and form interstitial oil conducting spaces.

FRANKLIN V. CHANEY.